

## UNITED STATES PATENT OFFICE

2,032,897

COATED ALUMINUM ARTICLE AND METHOD  
OF PRODUCING THE SAMERobert R. Tanner, Detroit, Mich., assignor to  
Metal Finishing Research Corporation, Detroit,  
Mich., a corporation of MichiganNo Drawing. Application October 31, 1934.  
Serial No. 759,747

3 Claims. (Cl. 148—6)

This invention relates to an article having a coated-aluminum surface and a method of producing that coating. More particularly, the invention relates to an article having an aluminum surface coated with aluminum fluoride, and aluminum fluoride produced in situ upon the surface, and to a method of producing said coated surface. An article presenting a surface of aluminum or an aluminum alloy may be coated for different reasons. The coating may be for purposes of resistance to corrosion, to facilitate coloring, as a foundation for paint or lacquer, to form electrical insulation, to affect the absorption, transmission or radiation of heat or light, or for other purposes.

By immersing the aluminum article in a weak solution of hydrofluoric acid substantially saturated with aluminum fluoride, a coating of aluminum fluoride may be formed in situ upon the aluminum surface. For example, in an aqueous solution containing 0.2% by weight of hydrofluoric acid and substantially saturated with aluminum fluoride, a very adherent coating can be formed at the boiling point in from 5 to 10 minutes. Such an aluminum fluoride coating is firmly adherent since it is formed substantially integrally with the subjacent metal. It also forms a base to which ordinary paint and lacquer adheres tenaciously, and in the event that the paint or lacquer becomes scratched at any point, the fluoride coating prevents any peeling off of the paint adjacent the scratch. Aluminum fluoride is very resistant, being substantially insoluble not only in water, but in ordinary alkalies, acids and alcohols. Therefore, it forms a permanent coating upon the aluminum surface which resists corrosion and forms a very good base for paint, lacquer or other finishing coatings which may be applied to give the article any desired appearance. It also has high electrical resistance, and modifies the conduction, absorption, reflection and emission of heat and like radiations.

While the solution of hydrofluoric acid does not form the fluoride coating until it has been substantially saturated with aluminum fluoride, it requires comparatively little aluminum fluoride to sufficiently saturate the dilute solution and therefore the solution may be allowed to dissolve the necessary amount of aluminum from the article when starting the coating operation unless a slight etching away of the article is unusually objectionable. In any case after a sufficiently dilute solution has been in use for a short time it becomes sufficiently saturated with aluminum fluoride so that the subsequent action thereof merely pro-

duces the surface coating upon the aluminum subjected thereto. This applies, of course, only where a solution of the order of dilution indicated above is employed. With stronger solutions, an etching rather than a coating action results, as discussed below.

One easy way to substantially saturate a dilute solution sufficiently for coating purposes is to allow the solution to act on aluminum powder or filings, but such a solution may be balanced, when preferred, by adding aluminum fluoride as such.

With a solution containing .2% hydrofluoric acid the addition of about .6% aluminum fluoride balances the solution sufficiently to produce a good coating. Increased amounts of the fluoride make possible the production of a coating with somewhat increased acidity, a strength of .5% acid having been used with good results; but increase of acidity above this point is needless, introduces difficulties, and soon reaches a point where it is practically impossible to balance the solution with aluminum fluoride so as to give satisfactory results. With too much acid, or without the balancing salt even with very dilute acid, only picking results. If the balancing aluminum fluoride is added as such, an excess should be avoided, as a solution within a good coating range of dilution below 1% gives only a very thin coloration or iridescence rather than a proper coating where an excess of aluminum fluoride is added.

Some other materials may be added to the solution for coloring or other purposes, and certain materials such as potassium permanganate, for example, may expedite the coating operation to some extent; but the coating operation may be easily inhibited by various foreign materials. There have been numerous proposals of solutions containing various amounts of hydrofluoric acid or compounds thereof for treatment of aluminum or compounds but so far as known these solutions have not been in such condition as to produce a coating of aluminum fluoride upon the surface of the aluminum. For example, the ordinary solution of hydrofluoric acid may be used to etch the surface of the aluminum, but as previously noted, it does not form a coating upon that surface until the solution is substantially saturated with aluminum fluoride, after which it has a coating rather than an etching action. In other words, wherever hydrofluoric acid is used for etching purposes, it obviously is not used for coating. Also, as previously noted, the hydrofluoric acid does not have a coating effect upon the aluminum in many combinations where other chemicals are

present which do have some coating effect upon the aluminum.

While the preferred solution is a very dilute solution of hydrofluoric acid substantially saturated with aluminum fluoride, it will be understood that broadly speaking, the invention covers various modifications which do not prevent the coating action which results in aluminum fluoride formed in situ upon the surface of the aluminum metal.

As indicated above, a coating formed in the manner specified forms a very good bonding coat for paint or lacquer, has electrical insulating properties, modifies the absorption, transmission reflection and radiation of heat, and is exceptionally resistant to corrosion. If desired the coating may be rendered very smooth by buffing.

While the thickness of the coating may vary with conditions and duration of the coating process, that normally produced has a thickness measurable by standard microscopic methods. In a typical instance, where two coated sheets were clamped together and the flush edges of the sheets treated to render the edges of the coatings visible, measurement by standard Bausch & Lomb microscopic measuring apparatus showed

a thickness for the two coatings of 0.0001 inch or one-half that for a single coating. A coating having a thickness of this order is quite effective for modifying the surface of the aluminum in the ways indicated, although thinner coatings may answer for some purposes and thicker coatings can be made if required.

What is claimed is:

1. A method of coating a metal surface, the major portion of which is metallic aluminum, which consists in immersing said surface in a hot dilute solution of hydrofluoric acid substantially saturated with aluminum fluoride.

2. An article having a metallic surface, the major portion of which consists of aluminum, covered with a substantially integral coating, the major portion of which consists of aluminum fluoride, said coating being of sufficient thickness for measurement by microscopic means.

3. An article having a metallic surface, the major portion of which consists of aluminum, covered with a substantially integral coating, the major portion of which consists of aluminum fluoride, said coating having a thickness of the order of 0.00005 inch.

25

ROBERT R. TANNER.